# EUROPEAN PATENT APPLICATION

(11) **EP 4 779 656 A1**
(43) Date of publication of application: **22.07.2026**
(21) Application number: 24878770.7
(22) Date of filing: 19.09.2024
(51) Int. Cl.: H01B 7/02, H01B 13/30, H01B 7/18, H01B 7/28, H01B 7/282, H01B 7/00, H01B 7/04, H01B 7/08, H01B 13/00, H01B 13/06

(54) **INSULATED WIRE, MANUFACTURING METHOD AND ELECTRICAL DEVICE**

(30) Priority: 19.10.2023 CN 202311361291
(71) Applicant: NINGBO JINTIAN ELECTROMAGNETIC TECHNOLOGY CO., LTD., Ningbo, Zhejiang 315336 (CN); NINGBO JINTIAN NEW MATERIAL CO., LTD., Ningbo, Zhejiang 315336 (CN)
(72) Inventor: GUO, Caifu, Hangzhou Bay New Area Ningbo, Zhejiang 315336 (CN); CHAI, Shoucun, Hangzhou Bay New Area Ningbo, Zhejiang 315336 (CN); ZHANG, Wei, Hangzhou Bay New Area Ningbo, Zhejiang 315336 (CN); DU, Changbin, Hangzhou Bay New Area Ningbo, Zhejiang 315336 (CN)
(74) Representative: Larsen & Birkeholm A/S
(86) International application number: PCT/CN2024/119603
(87) International publication number: WO 2025/082121

(57) **Abstract**

An insulated wire and a manufacturing method therefor, and an electrical device. The insulated wire comprises a wire and an insulating layer, wherein the insulating layer wraps the wire with at least one layer, and after being subjected to a minimum stretching of 15%, the insulated wire has a detachment distance of≤ the narrow side length of the wire. Using electromagnetic induction heating in the preheating stage enables the insulated wire to achieve uniform heating and stable temperature, which allows the insulating material to wrap the wire within the most suitable temperature range, and improves the adhesion between the insulating material and the wire during coating of the insulating material, thus increasing the bonding force, and improving the safety performance of an electrical device.

## Description

### CROSS REFERENCE TO RELATED APPLICATION

The present invention claims priority to Chinese Patent Application No. 202311361291.2, filed with the China National Intellectual Property Administration on October 19, 2023, which is incorporated herein by reference in entirety.

### TECHNICAL FIELD

The present invention relates to the technical field of inductance technology, specifically relates to an insulated wire and a manufacturing method therefor, and an electrical device.

### BACKGROUND ART

Insulated wires can be installed in any electrical appliance to conduct current without causing short circuits that could result from contact between non-electrically-insulated conductors. These insulated wires include a copper conductor and a coating of an insulated wire, typically including one layer or more layers.

However, in conventional insulated wires with preferably high-temperature resistant insulating layers, in particular, bonding force between an electrical conductor made of copper and an insulating coating is a matter of considerable concern at present, as plastics have a lower bonding force to electrical conductors due to their surface properties.

### SUMMARY

Therefore, the present invention provides an insulated wire and a manufacturing method therefor, and an electrical device. Using electromagnetic induction heating in the preheating stage enables the wire to be prepared at uniform heating and stable temperature, which allows the insulating material to wrap the wire within the most suitable temperature range, thereby increasing resilience and further facilitate to improve the adhesion between the insulating material and the wire during coating of the insulating material, thus increasing the bonding force, and improving the safety performance of an electrical device.

Therefore, the first objective of the present invention is to provide an insulated wire;
the second objective of the present invention is to provide a manufacturing method for an insulated wire; and
the third objective of the present invention is to provide an electrical device.

To achieve the first objective of the present invention, the present invention provides an insulated wire, wherein the insulated wire includes a wire and an insulating layer, wherein the insulating layer wraps the wire with at least one layer, and after being subjecting to a minimum elongation of 15%, the insulated wire's length of loss of adhesion is ≤ a narrow side length of the wire.

Compared with the prior art, the technical effects achieved by adopting the technical solution are as follows: the insulated wire consists of the wire and the insulating layer. The wire is used to conduct current, while the insulating layer can protect the wire from mechanical damage and chemical corrosion, prevent the wire from getting damp due to contact with water vapor, and avoid electric shock from contact with a conductor, etc., enhancing mechanical strength and extending service life, and reducing occurrence of safety accidents. Adhesion is one of factors for testing safety performance of an insulated wire. Typically, circular cutting is made perpendicular to an axis of a conductor on the insulated wire, the wire is subjected to stretching of 15%, and detachment between the insulating coating and an electric conductor is then measured. The less detachment between the insulating coating and the electric conductor is, the better the adhesion is. Since in the present invention, after being subjecting to a minimum elongation of 15%, the insulated wire's length of loss of adhesion is ≤ the narrow side length of the wire, indicating superior adhesion performance. Furthermore, improving the adhesion between the insulating material and the wire increases the bonding force of the insulated wire, improves effects of corrosion resistance, salt spray resistance, and chemical resistance, etc., prolongs service life of the insulated wire and improves safety performance of the insulated wire.

In a technical solution of the present invention, an elongation at break of the insulated wire is not less than 40%; and/or a springback angle of the insulated wire is 5.0°-5.5°; and/or a room temperature breakdown voltage of the insulated wire is not less than 16 kV.

Compared with the prior art, the technical effects achieved by adopting the technical solution are as follows: the elongation at break of the insulated wire is not less than 40%, indicating that the insulated wire has good plasticity and ductility when subjected to force, can absorb more energy, are more prone to deformation and will not break; the springback angle of the insulated wire is 5.0°-5.5°, and a small springback angle indicates a large degree of deformation, which is beneficial to the insulating material, but an excessively small springback angle may cause the insulating material to break. Therefore, selecting a springback angle of 5.0°-5.5° not only allows for a large degree of deformation of the insulating material, but also makes the insulating material less prone to be broken in subsequent use, thereby ensuring safety performance of an electrical device; and room temperature breakdown voltage of the insulated wire is not less than 16 kV. The higher the breakdown voltage is, the more uniform the electric field is and the longer the service life of the insulated wire is, thus obtaining an insulated wire with relatively superior performance.

In a technical solution of the present invention, the wire includes one or more selected from the group consisting of copper, oxygen-free copper, and copper alloys; and/or the insulating layer includes one or more selected from the group consisting of polyether ether ketone, modified polyether ether ketone, polyether ketone ketone, polyketone, polyphenylene sulfide, and thermoplastic polyimide; and/or the wire is flat/rectangular; and/or a thickness of the insulating layer is 80 µm-1200 µm; and/or a radius of any one of rounded corners of a cross-section of the insulated wire is 0.3 mm-2.0 mm; and/or a length of any one of sides of a cross-section of the insulated wire is 0.50 mm-20.00 mm.

Compared with the prior art, the technical effects achieved by adopting the technical solution are as follows: the wire includes one or more selected from the group consisting of copper, oxygen-free copper, copper alloy, and aluminum; a conductor is composed of copper or an alloy with high copper content, or aluminum, or other conductive materials, offering not only low cost but also excellent electrical conductivity; the insulating layer includes one or more selected from the group consisting of polyether ether ketone, modified polyether ether ketone, polyether ketone ketone, polyketone, polyphenylene sulfide, and thermoplastic polyimide; the insulating layer consists of at least one layer made of the above materials, providing better surface smoothness and flexibility; and high melting points of polyether ether ketone, modified polyether ether ketone, polyether ketone ketone, polyketone, polyphenylene sulfide, and thermoplastic polyimide ensure safety of the insulated wire; the wire is flat/rectangular, the thickness of the insulating layer is 80 µm-1200 µm, the radius of any one of rounded corners of a cross-section of the insulated wire is 0.3mm-2.0mm, the length of any one of sides of the cross-section of the insulated wire is 0.50 mm-20.00 mm, and a cross-section of an electrical conductor perpendicular to the axis of the conductor can be of any geometry: square, rectangular, circular, or elliptical, which is convenient for conduction, is easy to manufacture, and occupies smaller space in electrical appliances.

To achieve the second objective of the present invention, the present invention provides a manufacturing method for an insulated wire, used for manufacturing any one of the above insulated wires, wherein the manufacturing method includes following steps:
S100, subjecting a raw material of the wire to extrusion molding to obtain a flat/rectangular wire material;
S200, subjecting the flat/rectangular wire material to electromagnetic induction preheating by introducing a protective gas to obtain the wire; and
S300, heating and melting an insulating material to obtain an insulating melt; then coating the insulating melt on at least a portion of a surface of the wire, followed by a cooling treatment to obtain the insulated wire,
wherein the protective gas is a gas used to protect the material of the wire from oxidation.

Compared with the prior art, the technical effects achieved by adopting the technical solution are as follows: after the raw material of the wire was subjected to extrusion molding to obtain the flat/rectangular wire material, online electromagnetic induction preheating is performed simultaneously while introducing the protective gas, and the protective gas is a gas used to prevent the wire material from oxidation, preventing the wire from undergoing a chemical reaction with oxygen in the air during heating, which otherwise could lead to surface oxidation of the wire. Traditional heating method of insulating materials is performed by an oven treatment, resulting in inconsistency between a surface temperature and an internal temperature of the flat/rectangular wire material, that is, the internal temperature does not reach the surface temperature. However, electromagnetic heating achieves consistency between the surface temperature and a core temperature of the conductor. Electromagnetic heating reaches 135 °C-235 °C, enabling the insulating layer to bond the conductor tightly and easily, resulting in excellent adhesion performance of a product, thus increasing bonding force, thereby improving the safety performance of an electrical device. The insulating material is then heated and melted, and coated on a surface of the wire. Then, the insulating material is heated and melted, and coated on the surface of the wire, and as the wire has undergone the electromagnetic induction preheating, adhesion thereof is increased during coating, followed by a cooling treatment. A plane mirror is placed under the insulated wire to observe a color of a lower surface of the insulated wire and compare a color difference between an upper surface and a lower surface. Different colors represent different thicknesses of the insulating layer. By comparing the colors, it is possible to preliminarily determine whether there is a difference in the thickness of the insulating layer and make timely adjustments, and adjustment time can be greatly saved and generation of waste can be reduced.

**In** a technical solution of the present invention, in step S100, the extrusion molding is performed by using a cold extrusion mold; and/or a narrow-to-width ratio of the flat/rectangular wire material obtained by the extrusion molding is not less than 33%.

Compared with the prior art, the technical effects achieved by adopting the technical solution are as follows: the extrusion molding is performed by using the cold extrusion mold, and the mold needs to be designed according to the narrow-to-width ratio. Shapes of a narrow side and a wide side of the mold are not horizontal straight edges, but outward-protruding arcs. When the narrow-to-width ratio is less than 33% when the wire is in the extrusion process, uneven deformation and flow rate of the wire in a flat/rectangular hole type results in concave center point of the wide side of the extruded flat/rectangular wire, and uneven wide side of the extruded flat/rectangular copper wire, affecting flatness of the wire in subsequent production. Therefore, when the narrow-to-width ratio is less than 33%, the extrusion mold is designed as an outward-protruding arc shape, and a protrusion value is 0.020 mm-0.035 mm at the center of the wide side. When the narrow-to-width ratio is greater than 33%, the wide side does not need to protrude at the center. In addition, the smaller the narrow-to-width ratio is, the greater a required protrusion value of the wide side of the mold is. Based on practical considerations, when the narrow-to-width ratio of the flat/rectangular wire material obtained through extrusion molding is not less than 33%, various properties of the wire are optimal.

In a technical solution of the present invention, in step S200: a feed rate of the flat/rectangular wire material during the electromagnetic induction preheating is 2 m/min-9 m/min; and/or a temperature of the electromagnetic induction preheating is 135 °C-235 °C; and/or a pressure of the protective gas is 0.02 MPa-0.10 MPa.

Compared with the prior art, the technical effects achieved by adopting the technical solution are as follows: using electromagnetic induction to preheat the wire to 135°C -235°C enables the insulated wire to be prepared at uniform heating and stable temperature, which allows the insulating material to wrap the wire to achieve the optimal coating effect within the most suitable temperature range. Furthermore, controlling the feed rate of the flat/rectangular wire material being 2 m/min-9 m/min ensures that all parts of the wire reach preset heating temperatures during online electromagnetic heating, guaranteeing sufficient and uniform heating of the wire. Reasonable setting of the temperature of the electromagnetic induction heating and control of the feed rate can improve the adhesion between the insulating material and the wire during coating of the insulating material. Improving the adhesion between the insulating material and the wire further improves water resistance of the insulating material, improving corrosion resistance, salt spray resistance, and chemical resistance. Introducing protective gas during the electromagnetic induction preheating leads to an increase in pressure, but the pressure should not be too high, otherwise, it will to some extent lower surface temperature of the wire and cause inconsistent temperatures of the surface of the wire. Therefore, the pressure of the protective gas is set between 0.02 MPa-0.10 MPa.

In a technical solution of the present invention, before step S300, the manufacturing method further includes subjecting the insulating material to a drying treatment, wherein a duration of the drying treatment is 4 h-10 h; and/or a temperature of the drying treatment is 150 °C-160 °C.

Compared with the prior art, the technical effects achieved by adopting the technical solution are as follows: since the insulating material is generally in granular form, drying treatment is required before use. The duration of the drying treatment is 4 h-10 h and the temperature of the drying treatment is 150 °C-160 °C, achieving a completely dehumidified state and avoiding problems such as bubbles, surface wrinkling, unevenness, and roughness on a product surface, affecting subsequent production and use.

In a technical solution of the present invention, in step S300, a temperature of the heating and melting the insulating material includes four temperature zones; various temperature zones and corresponding temperatures are a temperature of a first temperature zone of 280°C-340°C, a temperature of a second temperature zone of 340°C-370°C, a temperature of a third temperature zone of 350°C-380°C, and a temperature of a fourth temperature zone of 360°C-390°C; and/or a temperature of the coating treatment is 370 °C-420 °C; and/or the cooling treatment is performed by using one or more of forced air cooling, natural air cooling, and water cooling.

Compared with the prior art, the technical effects achieved by adopting the technical solution are as follows: using a gradual heating method of multiple temperature zones better preserves performances of the insulating material than using a single-temperature heating method. Simultaneously, the service life of the insulating material is significantly prolonged, and wrapping property on the wire is more superior, improving toughness thereof and reducing hardness, making it suitable for large-scale production by enterprises. The temperature of the coating treatment is 370 °C-420 °C, and a melting point of the insulating material is 343 °C. Performing wrapping at a temperature higher than the melting point offers advantages of, on the one hand, better fluidity, and simpler coating operation, and one the other hand, better adhesion effect of coating, thus extending service life. The cooling treatment is performed by using one or more of forced air cooling, natural air cooling, and water cooling. Performing a gradient cooling treatment on a product after coating can solve product abnormality problems of poor surface quality or poor adhesion caused by excessively rapid cooling during the crystallization of the insulating material, thereby reducing industrial production costs.

In a technical solution of the present invention, after step S300, the manufacturing method further includes: sequentially performing optical detection processing and take-up processing on the insulated wire, wherein a speed of the take-up processing is 2 m/min-9 m/min.

Compared with the prior art, the technical effects achieved by adopting the technical solution are as follows: sequentially performing optical detection processing and take-up processing on the insulated wire, and promptly alarming for an over-limit situation, greatly improve detection and management of some of main product characteristics, reducing defective waste caused by poor high-voltage performance. Adjusting tension of the take-up processing and speed of the take-up processing is used for a neat arrangement of the taken-up wire and changing take-up reels, facilitating subsequent use.

To achieve the third objective of the present invention, the present invention provides an electrical device, including any one of the above insulated wires. Therefore, the beneficial effects that any one of the above technical solutions possesses will not be elaborated here.

The following technical effects can be achieved by adopting the technical solutions of the present invention:
(1) using electromagnetic induction heating in the preheating stage improves the adhesion between the insulating material and the wire during coating of the insulating material, thus increasing the bonding force, and improving the safety performance of an electrical device;
(2) performing the cooling treatment reduces product abnormality problems of poor surface quality or poor adhesion during the crystallization of the insulating material, and reduces industrial production costs, and the thickness of the insulating layer can be directly observed through a plane mirror. The thickness can be distinguished by color and adjusted in time, which can greatly save adjustment time and reduce waste generation; and
(3) adopting a cold extrusion mold treatment in the extrusion molding, and adjusting the narrow-to-width ratio of the wire to be not less than 33%, enables the resulting insulated wire to have excellent performance.

### BRIEF DESCRIPTION OF DRAWINGS

To more clearly illustrate the technical solutions of embodiments of the present invention, drawings that need to be used in the embodiments will be briefly introduced below. Obviously, the drawings below are only some embodiments of the present invention. For those ordinarily skilled in the art, other relevant drawings can be obtained based on these drawings without making any inventive efforts.
FIG. 1 is a flowchart of a manufacturing method for an insulated wire provided by an embodiment of the present invention.

### DETAILED DESCRIPTION OF EMBODIMENTS

To make the above objectives, features, and advantages of the present invention more obvious and understandable, the technical solutions in the embodiments of the present invention will be clearly and completely described. Obviously, the described embodiments are only some embodiments of the present invention, and not all embodiments. Based on the embodiments of the present invention, all other embodiments obtained by those ordinarily skilled in the art without making inventive efforts are within the scope of protection of the present invention.

An insulated wire can be installed in any electrical appliance to conduct current without causing short circuits that could result from contact between non-electrically-insulated conductors. The insulated wires include a copper conductor and a coating of the insulated wire, typically including one layer or more layers.

However, currently, in conventional insulated wires with preferably high-temperature resistant insulating layers, in particular, bonding force between an electrical conductor made of copper and an insulating coating is a matter of considerable concern at present, as plastics have a lower bonding force to electrical conductors due to surface properties.

Therefore, the present invention provides an insulated wire and a manufacturing method therefor, and an electrical device. Using electromagnetic induction heating in the preheating stage enables the insulated wire to achieve uniform heating and be prepared at a stable temperature, which allows the insulating material to wrap the wire within the most suitable temperature range, and improves the adhesion between the insulating material and the wire during coating of the insulating material, thus increasing the bonding force, and improving the safety performance of an electrical device. Furthermore, improving the adhesion between the insulating material and the wire further improves corrosion resistance, salt spray resistance, and chemical resistance of the insulated wire, thereby prolonging service life of the insulated wire.

Further, the elongation at break of the insulated wire is not less than 40%, indicating that the insulated wire has good plasticity and ductility when subjected to force, can absorb more energy, are more prone to deformation and will not break; the springback angle of the insulated wire is 5.0°-5.5°, and a small springback angle indicates a large degree of deformation, which is beneficial to the insulating material, but an excessively small springback angle may cause the insulating material to break. Therefore, selecting a springback angle of 5.0°-5.5° not only allows for a large degree of deformation of the insulating material but also makes the insulating material less prone to be broken in subsequent use, thereby ensuring safety performance of an electrical device; and room temperature breakdown voltage of the insulated wire is not less than 16 kV. The higher the breakdown voltage is, the more uniform the electric field is and the longer the service life of the insulated wire is, thus obtaining an insulated wire with relatively superior performance. A specific manufacturing method is as follows.

First, the wire raw material is subjected to extrusion molding to obtain a flat/rectangular wire material; and the flat/rectangular wire material is then subjected to electromagnetic induction preheating by introducing a protective gas to obtain the wire.

Preferably, the extrusion molding is performed by using a cold extrusion mold to obtain a flat/rectangular wire material with a narrow-to-width ratio less than 33%. Shapes of a narrow side and wide side of the mold are horizontal straight edges. Uneven deformation and flow rate of the wire in a flat/rectangular hole type of the mold results in concave center point of the wide side of the extruded flat/rectangular wire, and uneven wide side of the extruded flat/rectangular copper wire, affecting flatness of the wire in subsequent production. Therefore, when the narrow-to-width ratio is less than 33%, the wide side of the extrusion mold is designed as an outward-protruding arc shape, and when the narrow-to-width ratio is less than 33%, a protrusion value needs to be 0.020 mm-0.035 mm at the center of the wide side. When the narrow-to-width ratio is greater than 33%, the wide side does not need to protrude at the center. In addition, the smaller the narrow-to-width ratio is, the greater a required protrusion value of the wide side of the mold is. Based on practical considerations, when the narrow-to-width ratio of the flat/rectangular cooper wire material obtained through extrusion molding is not less than 33%, various properties of the wire are optimal.

Further, the protective gas is a gas used to prevent the wire material from oxidation, preventing the wire from undergoing a chemical reaction with oxygen in the air during heating, which otherwise could lead to surface oxidation of the wire. Traditional heating method of insulating materials is performed by an oven treatment, resulting in inconsistency between a surface temperature and an internal temperature of the flat/rectangular wire material, that is, the internal temperature does not reach the surface temperature. However, electromagnetic heating achieves consistency between the surface temperature and a core temperature of the conductor. Electromagnetic heating reaches 135 °C-235 °C, achieving optimal coating effects through matching of a temperature of the wire with a temperature of the insulated material. Furthermore, controlling the feed rate of the flat/rectangular wire material of 2 m/min-9 m/min ensures that all parts of the wire reach preset heating temperatures during online electromagnetic heating, guaranteeing sufficient and uniform heating of the wire. Reasonable setting of the temperature of the electromagnetic induction heating and control of the feed rate can improve the adhesion between the insulating material and the wire during coating of the insulating material, further improving water resistance of the insulating material, and improving corrosion resistance, salt spray resistance, and chemical resistance. Introducing protective gas during the electromagnetic induction preheating leads to an increase in pressure, but the pressure should not be too high, otherwise, it will to some extent lower surface temperature of the wire and cause inconsistent temperatures of the surface of the wire. Therefore, the pressure of the protective gas is set between 0.02 MPa-0.10 MPa.

Subsequently, the insulating material is heated and melted to obtain an insulating melt; then the insulating melt is subjected to a coating treatment on at least a portion of a surface of the wire, followed by a cooling treatment to obtain the insulated wire.

Preferably, the insulating material is heated and melted and then coated onto the surface of the wire. Since the wire has undergone the electromagnetic induction preheating, adhesion thereof can be increased during coating. Furthermore, improving the adhesion between the insulating material and the wire further improves the bonding force of the insulated wire, improving corrosion resistance, salt spray resistance, and chemical resistance, prolonging service life of the insulated wire, and improving safety performance of the insulated wire.

Further, cooling treatment is performed, and the cooling treatment is performed by using one or more of forced air cooling, natural air cooling, and water cooling. A gradient cooling treatment is performed to solve product abnormality problems of poor surface quality or poor adhesion caused by excessively rapid cooling during the crystallization of the insulating material, thereby reducing industrial production costs. Meanwhile, a plane mirror can be placed under the insulated wire to observe a color of a lower surface of the insulated wire and compare a color difference between an upper surface and a lower surface. Different colors represent different thicknesses of the insulating layer. By comparing the colors, it is possible to preliminarily determine whether there is a difference in the thickness of the insulating layer and make timely adjustments, and adjustment time can be greatly saved and generation of waste can be reduced. The darker the color is, the thinner the coating is and the lighter the color is, the thicker the coating is.

Further, optical detection processing and take-up processing on the insulated wire are sequentially performed, wherein a speed of the take-up processing is 2 m/min-9 m/min; Sequentially performing optical detection processing and take-up processing on the insulated wire, and promptly alarming for an over-limit situation, greatly improve detection accuracy and management of some of main product characteristics, reducing defective waste caused by poor high-voltage performance. Adjusting tension of the take-up processing and speed of the take-up processing is used for a neat arrangement of the taken-up wire and changing take-up reels, facilitating subsequent use.

### Example 1

The present example provided a manufacturing method for an insulated wire. A flowchart for the manufacturing method is shown in FIG. 1, and specific operation steps were as follows:
S100, a copper wire was subjected to extrusion molding using a cold extrusion mold to obtain a flat/rectangular copper wire with a length of a side of a cross-section of 1.990 mm × 3.060 mm, a narrow-to-width ratio of 65%, and a radius of a rounded corner of a cross-section of 0.40 mm;
S200, in a protective gas, the flat/rectangular wire material was passed through a preheated pipe at a feed rate of 2 m/min, with a set temperature of 135 °C and an output pressure of the protective gas of 0.02 MPa for electromagnetic induction preheating to obtain the wire; and
S300, a Peek material (polyether ether ketone) was heated and melted in a first temperature zone of 280 °C, a second temperature zone of 340 °C, a third temperature zone of 350 °C, and a fourth temperature zone of 360 °C, to obtain a Peek material (polyether ether ketone) melt; the Peek material (polyether ether ketone) melt was then coated on at least a portion of a surface of the wire at 370 °C, followed by performing a gradient cooling treatment by combining forced air cooling and natural air cooling to obtain the insulated wire with an insulating layer with a thickness of a side of the rounded corner of 150 µm, a thickness of a wide side of 148 µm, a thickness of a narrow side of 150 µm, and a radius of the rounded corner of a cross-section of 0.57 mm;
wherein the protective gas was nitrogen, and the Peek material (polyether ether ketone) was dried in an oven at 150 °C for 8 h. After obtaining the insulated wire, optical detection processing and take-up processing were performed sequentially, wherein a speed of the take-up processing was 2 m/min.

### Example 2

The present example provided a manufacturing method for an insulated wire, as shown in FIG. 1, and specific operation steps were as follows:
S100, a copper alloy wire was subjected to extrusion molding using a cold extrusion mold to obtain a flat/rectangular copper wire with a length of a side of a cross-section of 0.700 mm × 1.040 mm, a narrow-to-width ratio of 67%, and a radius of a rounded corner of a cross-section of 0.3 mm;
S200, in a protective gas, the flat/rectangular wire material was passed through a preheated pipe at a feed rate of 5 m/min, with a set temperature of 200 °C and an output pressure of the protective gas of 0.1 MPa for electromagnetic induction preheating to obtain a wire; and
S300, a Peek material (modified polyether ether ketone) was heated and melted in a first temperature zone of 300 °C, a second temperature zone of 360 °C, a third temperature zone of 370 °C, and a fourth temperature zone of 380 °C, to obtain a Peek material (polyether ether ketone) melt; the Peek material (polyether ether ketone) melt was then coated on at least a portion of a surface of the wire at 400 °C, followed by performing a gradient cooling treatment by combining forced air cooling and natural air cooling to obtain the insulated wire with an insulating layer with a thickness of a side of the rounded corner of 80 µm, a thickness of a wide side of 80 µm, a thickness of a narrow side of 80 µm, and a radius of the rounded corner of a cross-section of 0.4 mm,
wherein the protective gas was argon, and the Peek material (polyether ether ketone) was dried in an oven at 160 °C for 10 h. After obtaining the insulated wire, optical detection processing and take-up processing were performed sequentially, wherein a speed of the take-up processing was 5 m/min.

### Example 3

The present example provided a manufacturing method for an insulated wire, as shown in FIG. 1, and specific operation steps were as follows:
S100, a copper alloy wire was subjected to extrusion molding using a cold extrusion mold to obtain a flat/rectangular copper wire with a length of a side of a cross-section of 4.440 mm × 12.000 mm, a narrow-to-width ratio of 37%, and a radius of a rounded corner of a cross-section of 2 mm;
S200, in a protective gas, the flat/rectangular wire material was passed through a preheated pipe at a feed rate of 9 m/min, with a set temperature of 235 °C and an output pressure of the protective gas of 0.1 MPa for electromagnetic induction preheating to obtain the wire; and
S300, a Peek material (polyether ether ketone) was heated and melted in a first temperature zone of 340 °C, a second temperature zone of 370 °C, a third temperature zone of 380 °C, and a fourth temperature zone of 390 °C, to obtain a Peek material (polyether ether ketone) melt; the Peek material (polyether ether ketone) melt was then coated on at least a portion of a surface of the wire at 420 °C, followed by performing a gradient cooling treatment by combining forced air cooling and natural air cooling to obtain the insulated wire with an insulating layer with a thickness of a side of the rounded corner of 1200 µm, a thickness of a wide side of 1200 µm, a thickness of a narrow side of 1200 µm, and a radius of rounded corners of a cross-section of 2.2 mm,
wherein the protective gas was helium, and the Peek material (polyether ether ketone) was dried in an oven at 160 °C for 10 h. After obtaining the insulated wire, optical detection processing and take-up processing were performed sequentially, wherein a speed of the take-up processing was 9 m/min.

### Comparative Example 1

The present invention provided a manufacturing method for an insulated wire. Specific operation steps were detailed in Example 1. A difference was that in step S200, the oven treatment was performed for preheating.

### Comparative Example 2

The present comparative example provided a manufacturing method for an insulated wire. Specific operation steps were detailed in Example 1. A difference was that in S300, the Peek material (polyether ether ketone) was heated and melted at a temperature of 360 °C to obtain the Peek material (polyether ether ketone) melt without stage heating.

### Comparative Example 3

The present comparative example provided a manufacturing method for an insulated wire. Specific operation steps were detailed in Example 1. A difference was that in step S200, a protective gas was not introduced during electromagnetic induction preheating.

Performance tests were conducted on Examples 1-3 and Comparative Examples 1-3. Specific steps were as follows, and experimental results are shown in Table 1.

Test steps of the adhesion of the insulated wire were as follows:
① a sample of approximately 300 mm was taken for straightening;
② the sample was placed parallel to and tightly against a steel ruler and a section with a length of 200 mm at a straight part was taken and an original gauge length was marked using a marker. At the middle of the gauge length, a cut was made around the sample with a knife until the copper conductor was exposed;
③ the sample was fixed on a tensile testing machine and stretched by 15% at a speed of 5±1 mm/s; and
④ the sample was taken and a distance at which it loses its adhesion to the conductor was measured from the cut line along the longitudinal direction on each side of the sample using a microscope. A maximum length of detachment for a single sample was recorded.

Test steps of an elongation at break of the insulated wire were as follows:
① three samples of approximately 300 mm in length were taken for straightening;
② the samples were placed parallel to and tightly against a steel ruler and a section with a length L1 of 200 mm at the straight part was taken and the original gauge length was marked using a marker;
③ the samples were fixed on a tensile testing machine and stretched until fracture at a speed of 5±1 mm/s; and
④ two broken samples were taken and the two broken samples were brought into close contact at fracture ends, and a distance L2 between the original marks was measured with a ruler. The elongation at break of the insulated wire was calculated by dividing length data L2 by the marked length data L1 before stretching and then subtracting 1.

Test steps of resistivity of the insulated wire at 20 °C were as follows:
① a sample with a length of 1 m was taken, coating films at both ends were removed by a method without damaging the copper material, and the sample was then left to stand at 20°C-25 °C for 1 h; and
② a resistance of the sample with a length of 1 m at 20 °C was measured using a high-precision resistance tester.

Test steps of the springback angle of the insulated wire were as follows:
① three samples of approximately 400 mm were taken for straightening, with a free end extending 12±2 mm beyond a slider notch;
② a slider distance of 40 times the narrow side dimension L = 96.8 mm was calculated;
③ a handle was bended from 30° to 0° within 2-5 s, with a maximum standing duration of 2 s, and the handle was retracted in an opposite direction at the same speed until the notch slid away from the sample;
④ the sample was allowed to spring back freely and stabilized; the handle was moved again until just touching the sample without bending the sample; and an angle, i.e., the springback angle was read on a sector scale; and
⑤ the measurement was repeated three times and an average value was taken as the test result.

Test steps of a room temperature breakdown voltage of the insulated wire were as follows:
① 5 samples of 400 mm were taken for straightening; and the wide side was blended by 180° using a round rod with a diameter of 25 mm;
② a "U"-shaped bend was placed into steel balls with a diameter of 2 mm and the wires were connected according to the requirements; and
③ a voltage tester was started; the equipment automatically tested the 5 samples and recorded breakdown voltages of the 5 samples.

Test steps of PDIV of the insulated wire were as follows:
① 5 pieces of back-to-back samples were prepared according to the requirements and allowed to stand for 1 h in an environment with a temperature of 20 °C-25 °C and a humidity of 45%-55%;
② the samples were connected to equipment and parameters were set according to following requirements: power frequency sinusoidal wave frequency of 50 Hz; voltage rise rate of 50 V/s; and discharge magnitude of 100 pc; and
③ values of partial discharge inception voltage were measured and recorded.

**Table 1**

| [Table 1_sm_0001] | | | | | | |
|---|---|---|---|---|---|---|
| Item | Example 1 | Example 2 | Example 3 | Comparative Example 1 | Comparative Example 2 | Comparative Example 3 |
| Adhesion (mm) | 1.3 | 0.4 | 1.9 | 3.1 | 1.9 | 2.2 |
| Elongation at Break (%) | 45 | 43 | 44 | 41 | 41 | 40 |
| Resistivity (C) at 20 °C | 0.01701 | 0.01697 | 0.01697 | 0.01702 | 0.01699 | 0.01701 |
| Springback Angle | 5.3 | 5.2 | 5.0 | 5.2 | 5.1 | 5.2 |
| Room Temperature Breakdown Voltage (KV) | 17.3 | 16.4 | 17.5 | 15.2 | 15.7 | 14.8 |
| PDIV (V) | 1750 | 1831 | 1956 | 1831 | 1602 | 1856 |

Finally, it should be noted that the above embodiments are only used to illustrate the technical solutions of the present invention and are not intended to limit thereof. Although the present invention has been described in detail with reference to the above embodiments, those ordinarily skilled in the art should understand that: modifications can still be made to the technical solutions of the above embodiments, or equivalent substitutions can be made to some of the technical features; and these modifications or substitutions do not cause the essence of corresponding technical solutions to deviate from the spirit and scope of the technical solutions of the embodiments of the present invention.

## Claims

1. An insulated wire, **characterized in that** the insulated wire comprises:
a wire; and
an insulating layer, wherein the insulating layer wraps the wire with at least one layer, wherein
after being subjecting to a minimum elongation of 15%, the insulated wire's length of loss of adhesion is ≤ a narrow side length of the wire.

2. The insulated wire according to claim 1, wherein
an elongation at break of the insulated wire is not less than 40%; and/or
a springback angle of the insulated wire is 5.0°-5.5°; and/or
a room temperature breakdown voltage of the insulated wire is not less than 16 kV.

3. The insulated wire according to claim 1, wherein
the wire comprises one or more selected from the group consisting of copper, oxygen-free copper, and copper alloys; and/or
the insulating layer comprises one or more selected from the group consisting of polyether ether ketone, modified polyether ether ketone, polyether ketone ketone, polyketone, polyphenylene sulfide, and thermoplastic polyimide; and/or
the wire is flat/rectangular; and/or
a thickness of the insulating layer is 80 µm-1200 µm; and/or
a radius of any one of rounded corners of a cross-section of the insulated wire is 0.3 mm-2.0 mm; and/or
a length of any one of sides of a cross-section of the insulated wire is 0.50 mm-20.00 mm.

4. A manufacturing method for an insulated wire, for preparing the insulated wire according to any one of claims 1 to 3, **characterized in that** the manufacturing method comprises following steps:
S100, subjecting a raw material of the wire to extrusion molding to obtain a flat/rectangular wire material;
S200, subjecting the flat/rectangular wire material to electromagnetic induction preheating by introducing a protective gas to obtain the wire; and
S300, heating and melting an insulating material to obtain an insulating melt; then coating the insulating melt on at least a portion of a surface of the wire, followed by a cooling treatment to obtain the insulated wire,
wherein the protective gas is a gas used to protect the material of the wire from oxidation.

5. The manufacturing method according to claim 4, wherein in step S100:
the extrusion molding is performed by using a cold extrusion mold; and/or
a narrow-to-width ratio of the flat/rectangular wire material obtained by the extrusion molding is not less than 33%.

6. The manufacturing method according to claim 4, wherein in step S200:
a feed rate of the flat/rectangular wire material during the electromagnetic induction preheating is 2 m/min-9 m/min; and/or
a temperature of the electromagnetic induction preheating is 135 °C-235 °C; and/or
a pressure of the protective gas is 0.02 MPa-0.10 MPa.

7. The manufacturing method according to claim 4, before step S300, further comprising:
subjecting the insulating material to a drying treatment;
a duration of the drying treatment is 4 h-10 h; and/or
a temperature of the drying treatment is 150 °C-160 °C.

8. The manufacturing method according to claim 4, wherein in step S300:
a temperature for heating and melting the insulating material comprises four temperature zones; various temperature zones and corresponding temperatures are a temperature of a first temperature zone of 280 °C-340 °C, a temperature of a second temperature zone of 340 °C-370 °C, a temperature of a third temperature zone of 350 °C-380 °C, and a temperature of a fourth temperature zone of 360 °C-390 °C; and/or
a temperature of the coating treatment is 370 °C-420 °C; and/or
the cooling treatment is performed by using one or more of forced air cooling, natural air cooling, and water cooling.

9. The manufacturing method according to claim 4, after step S300, further comprising:
sequentially performing optical detection processing and take-up processing on the insulated wire,
wherein a speed of the take-up processing is 2 m/min-9 m/min.

10. An electrical device, **characterized by** comprising the insulated wire according to any one of claims 1 to 3.
